

# United States Patent Office

3,117,037

Patented Jan. 7, 1964

1

3,117,037

## PRODUCTION OF HIGH STRENGTH STEEL STRUCTURAL SHAPES

John M. Hodge, Pleasant Hills, Pa., assignor to United States Steel Corporation, a corporation of New Jersey  
No Drawing. Filed Sept. 22, 1961, Ser. No. 139,871  
5 Claims. (Cl. 148—12.3)

This invention relates to the production of structural steel shapes formed of high strength steel and more particularly to a method of forming straight, high strength, steel structural shapes.

In many structures such as bridges, towers, transportation and storage equipment there is a need for structural shapes having high strength. If structural shapes, such as beams, channels and angles having yield strengths in excess of 80,000 p.s.i. were available, a considerable reduction in weight could be obtained in such structures and along therewith reduced costs. Heretofore many attempts have been made to produce high strength in such structural shapes by resorting to conventional quenching and tempering. That is to say the high strengths were produced by drastically quenching the shapes formed of hardenable steel from an austenitizing temperature. While desired mechanical properties can be so obtained, the abrupt transformation or change in microstructure produces distortion so that the shapes have excessive camber, sweep, or twist or other distortion defects. Due to the high strength of such shapes, straightening by conventional straightening methods is very uneconomical and difficult and moreover has a deleterious effect on the mechanical properties of the steel.

It is accordingly an object of the present invention to produce undistorted and straight structural shapes of high strength steel.

It is a further object to produce such shapes in an efficient and economical manner.

I have discovered a method of producing structural shapes having strengths and properties comparable to quenched and tempered shapes and which are within commercial straightness tolerances. Successful utilization of the method of my invention requires the use of a low-carbon steel having a sufficiently high hardenability that it will obtain the desired hardness air cooling on a conventional hot-bed. Steel within the following compositional limits is satisfactory for practicing my invention:

|            | Percent   |
|------------|-----------|
| Carbon     | .15/.20   |
| Manganese  | .20/.50   |
| Silicon    | .15/.35   |
| Nickel     | 2.50/4.25 |
| Chromium   | 1.30/2.00 |
| Molybdenum | .35/.55   |

with the balance iron, residual impurities and other elements in amounts which do not deleteriously affect the properties.

Within such ranges, I have two preferred compositions as follows:

Table I

|            | A         | B         |
|------------|-----------|-----------|
| Carbon     | .15/.20   | .15/.20   |
| Manganese  | .20/.45   | .20/.45   |
| Silicon    | .15/.30   | .15/.30   |
| Nickel     | 2.75/3.25 | 3.75/4.25 |
| Chromium   | 1.60/1.90 | 1.70/2.00 |
| Molybdenum | .40/.60   | .40/.65   |

balance iron and residual impurities.

In accordance with my invention, structural shapes are

2

rolled from such steels by conventional practice and while at hot-rolling temperatures and in an austenitic condition are straightened, preferably by roller straightening, directly following the hot-rolling. After straightening 5 while in an austenitic condition the shapes are placed on conventional hot-beds and cooled to room temperature. During cooling, the steel transforms to a structure of lower bainite and martensite and because of the slow cooling rate is essentially straight due to lack of distortion during cooling and transformation. Any slight 10 distortions at this stage can easily be removed by gag-press or the like straightening. However, the cooling rate is sufficiently fast to produce a structure of lower bainite and martensite. Following transformation on the hot-bed, the sections have the desired high strength but due 15 to the presence of martensite may be lacking in toughness so that I prefer a final tempering step.

As an example of my invention, I have produced structural sections of steel of the following composition:

|            | Percent |
|------------|---------|
| Carbon     | .15     |
| Manganese  | .26     |
| Silicon    | .25     |
| 25 Nickel  | 2.95    |
| Chromium   | 1.83    |
| Molybdenum | .48     |

After hot-rolling, the sections were roller-straightened, 30 cooled on a hot-bed to room temperature and thereafter tempered at 1225° F. The sections were straight within commercial tolerances. Mechanical properties of three different sections so produced were as follows:

35

Table II

| Section | Yield Strength<br>(0.2% Offset),<br>p.s.i. | Tensile Strength,<br>p.s.i. | Elongation in<br>2", per<br>cent | Reduction of<br>Area,<br>Percent | V-Notch Charpy<br>Impact, ft./lb. |           |            |
|---------|--------------------------------------------|-----------------------------|----------------------------------|----------------------------------|-----------------------------------|-----------|------------|
|         |                                            |                             |                                  |                                  | Room<br>Temp.                     | -40<br>F. | -120<br>F. |
| 1       | 93,800                                     | 113,200                     | 28.8                             | 54.2                             | 85                                | 73        | 39         |
| 2       | 98,500                                     | 119,600                     | 25.0                             | 50.3                             | 72                                | 45        | 25         |
| 3       | 94,200                                     | 115,300                     | 21.2                             | 65.5                             | 85                                | 50        | 27         |

As can be seen, these properties are equivalent to those obtained by quenching and tempering, including high strength and toughness. Moreover, the sections were straight within commercial tolerances as produced.

While I have shown and described several specific embodiments of my invention, it will be understood that these embodiments are merely for the purpose of illustration and description and that various other forms may be devised within the scope of my invention, as defined in the appended claims.

I claim:

1. A method of producing high strength steel structural sections such as beams, channels and angles comprising hot-rolling sections of low-carbon steel having sufficiently high hardenability that it will harden during air cooling on a hot-bed, straightening said sections after hot-rolling and prior to cooling below the temperature at which the steel is austenitic, air cooling said sections to room temperature on a hot-bed at a rate sufficiently slow that distortion due to abrupt transformation does not occur but at a rate sufficiently fast to produce a martensitic-bainitic structure therein and thereafter tempering said sections at a temperature below the lower critical temperature thereof.
2. A method of producing high strength steel structural

sections such as beams, channels and angles comprising forming sections of steel of the following composition:

|            | Percent   |
|------------|-----------|
| Carbon     | .15/ .20  |
| Manganese  | .20/ .50  |
| Silicon    | .15/ .35  |
| Nickel     | 2.50/4.25 |
| Chromium   | 1.30/2.00 |
| Molybdenum | .35/ .55  |

with the balance iron, residual impurities and other elements in amounts which do not deleteriously affect the properties, straightening said sections after hot-rolling and before cooling below an austenitizing temperature, air cooling the straightened sections at a cooling rate sufficiently slow to prevent distortion therein but at a rate sufficiently fast to produce a transformation of the structure of the steel to lower bainite and martensite and thereafter tempering the sections at a temperature below the critical temperature thereof.

3. A method of producing high strength steel structural sections such as beams, channels and angles comprising forming sections of steel of the following composition:

|            | Percent   |
|------------|-----------|
| Carbon     | .15/ .20  |
| Manganese  | .20/ .45  |
| Silicon    | .15/ .30  |
| Nickel     | 2.75/3.25 |
| Chromium   | 1.60/1.90 |
| Molybdenum | .40/ .60  |

balance iron and residual impurities, roller straightening said sections after hot-rolling and before cooling below an austenitizing temperature, air cooling the straightened sections on a hot-bed at a cooling rate sufficiently slow to prevent distortion therein but at a rate sufficiently fast to produce a transformation of the structure of the steel to lower bainite and martensite and thereafter tempering the sections at a temperature below the critical temperature thereof.

4. A method of producing high strength steel structural sections such as beams, channels and angles comprising forming sections of steel of the following composition:

|            | Percent   |
|------------|-----------|
| Carbon     | .15/ .20  |
| Manganese  | .20/ .45  |
| Silicon    | .15/ .30  |
| Nickel     | 3.75/4.25 |
| Chromium   | 1.75/2.00 |
| Molybdenum | .40/ .65  |

balance iron and residual impurities, roller straightening said sections after hot-rolling and before cooling below an austenitizing temperature, air cooling the straightened sections on a hot-bed at a cooling rate sufficiently slow to prevent distortion therein but at a rate sufficiently fast to produce a transformation of the structure of the steel to lower bainite and martensite and thereafter tempering the sections at a temperature below the critical temperature thereof.

5. A method of producing high-strength structural shapes such as beams, channels and angles comprising hot-rolling structural shapes from steel containing

|            | Percent    |
|------------|------------|
| Carbon     | About .15  |
| Manganese  | About .26  |
| Silicon    | About .21  |
| Nickel     | About 2.95 |
| Chromium   | About 1.83 |
| Molybdenum | About .48  |

with the balance iron and residual impurities, hot-roller straightening said sections at the finish of the hot-rolling and before the sections have cooled below an austenitizing temperature, air cooling said sections on a hot-bed to produce straight sections having a lower bainite, martensitic structure therein and then tempering said sections at a temperature of about 1225° F.

35 References Cited in the file of this patent

UNITED STATES PATENTS

|           |               |               |
|-----------|---------------|---------------|
| 976,891   | Machlet       | Nov. 29, 1910 |
| 2,003,094 | Shimer et al. | May 28, 1935  |
| 2,087,346 | Johnston      | July 20, 1937 |
| 2,088,282 | Van Royen     | July 27, 1937 |

FOREIGN PATENTS

|         |               |                |
|---------|---------------|----------------|
| 344,822 | Great Britain | Mar. 11, 1931  |
| 472,464 | Great Britain | Sept. 16, 1937 |

UNITED STATES PATENT OFFICE  
CERTIFICATE OF CORRECTION

Patent No. 3,117,037

January 7, 1964

John M. Hodge

It is hereby certified that error appears in the above numbered patent requiring correction and that the said Letters Patent should read as corrected below.

Column 1, line 44, after "hardness" insert -- during --;  
column 4, line 6, for "1.75/2.00" read -- 1.70/2.00 --.

Signed and sealed this 26th day of May 1964.

(SEAL)

Attest:

ERNEST W. SWIDER  
Attesting Officer

EDWARD J. BRENNER  
Commissioner of Patents